

## 1

2,912,386

CORROSION INHIBITOR BY MEANS OF  
1,2-DITHIOLANES

Paul L. Salzberg, Wilmington, Del., assignor to E. I. du Pont de Nemours and Company, Wilmington, Del., a corporation of Delaware

No Drawing. Application August 1, 1957  
Serial No. 675,578

6 Claims. (Cl. 252—395)

This invention is concerned with the prevention of corrosion of metals, especially corrosion caused by acidic aqueous media. More particularly, the invention relates to a method for reducing the corrosive effect of an acidic composition in contact with an iron-containing metallic substance utilizing as corrosion inhibitors certain substituted 1,2-dithiolanes and their derivatives.

In the packaging of moist, wet or liquid materials in metal containers, a major concern is the prevention of corrosion of the metal with resultant contamination of the contents and destruction of the container. This is particularly true of packaged foods inasmuch as a large proportion of such foods are acidic, that is, have a pH below 7, and are highly corrosive to most metals.

For economic reasons, sheet steel is a desirable base from which to form containers and many means have been employed to reduce its corrosion by acidic media. Plating the steel with tin and coating either the steel or the tin-plated steel with resinous organic coatings represent well-known methods for protecting the base metal of a metal container. Such containers are satisfactory for many kinds of aqueous acidic products. However, certain acidic foods, particularly carbonated beverages, are difficult to preserve, even in tin-plated metal containers which have an additional resinous topcoat. This is so because it is extremely difficult to eliminate all pin holes from the various coatings, and corrosion of the base metal becomes a hazard. Consequently, means for preventing corrosion of metal containers by aqueous acidic contents are constantly being sought by workers in the container field.

It has now been found that the corrosive effect of an acidic composition in contact with an iron-containing metal can be reduced by a method which comprises including in said composition from 0.0001 to 10% by weight thereof of an organic compound of molecular weight not exceeding 500 and of the formula R—R'—COR", wherein R is a monovalent organic radical of the class consisting of



and the C-alkyl derivatives of these radicals wherein the alkyl groups are up to four carbons, R' is a divalent hydrocarbon radical of up to eight carbon atoms, R'' and R''' can be the same or different and singly represent hydrogen or a hydrocarbon radical containing up to 10 carbon atoms and taken together represent a divalent hydrocarbon radical having not more than 20 carbon atoms, and COR" is selected from the class consisting of carboxyl and groups hydrolyzable thereto. The R'' substituent in the grouping —COR" is preferably hydroxy, amido, lower alkoxy or an alkali metal such as sodium. However, other metal salts, ammonium salts, N-substituted amides and long-chain esters such as octadecyl can be

## 2

used and fall within the scope of this invention. It will be understood that the term "metal" is used herein in its broadest sense and includes mixed metals or alloys as well as metals in the elementary sense.

5 This invention also contemplates the product produced in employing the above method. In other words, my invention is also directed to a manufacture comprising an iron-containing metal container having therein an acidic commodity and from 0.0001 to 10% by weight of the 10 commodity of an organic compound of molecular weight not exceeding 500 and of the formula R—R'—COR", as defined above.

The iron-containing metals which are protected from corrosion by the present invention include cast iron, ingot 15 iron, wrought iron, low carbon, medium carbon, and high carbon steels, and alloy steels containing 50% or more iron by weight. The examples which follow employ a representative type of this group of iron-containing metals designated as black iron or black plate. This is a thin 20 rolled sheet steel with an iron content above 98.5% which is widely used as a base for "tin" can manufacture.

In a preferred embodiment of this invention, an acidic commodity, such as ginger ale or vinegar, is modified by the addition of 0.1% by weight of  $\alpha$ -lipoic acid, i.e., 25 5-(1,2-dithiolan-3-yl)pentanoic acid. The resulting acidic commodity is packaged in a clean, uncoated, black plate steel can. The resulting manufacture shows no corrosion of the inner surface of the can when opened after several weeks of storage at room temperature.

30 The following examples, in which parts are by weight except where otherwise indicated, are intended for the purpose of illustrating the invention. It will be appreciated that the examples are not intended to limit the invention, since the invention is susceptible to modification without departure from the letter and spirit of the 35 appended claims.

## Example 1

A sample of commercial ginger ale ("Canada Dry") is divided into two portions. Portion A is modified by the 40 addition of 10 p.p.m. (parts per million) of dl- $\alpha$ -lipoic acid. Portion B is unmodified. The two portions are placed in separate glass containers. In each container is placed a 3" x 1" panel of black iron sheet degreased by vapor treatment with trichloroethylene immediately prior to immersion in the ginger ale. The containers are only partly filled, the upper portions containing air, and are capped lightly to prevent evaporation. After storage at room temperature for thirteen days, the metal panel in 45 sample A is bright and the liquid only slightly discolored; whereas, the metal panel in sample B is discolored and the liquid is dark brown.

## Example 2

Black iron panels are washed with benzene, sanded, 55 washed with acetone, and air dried prior to immersion in the following solutions. Solution C is a sample of commercial ginger ale ("Canada Dry") having added thereto 100 p.p.m. of dl- $\alpha$ -lipoic acid, and solution D is a portion of the same ginger ale without the lipoic acid. The 60 solutions and panels are stored in glass containers with vented caps. After 3½ months at room temperature, the metal in sample C retains its full brightness and the liquid shows no discoloration. In sample D, the metal is discolored and the liquid is dark brown.

## Example 3

Three bottles of a commercial ginger ale ("Canada Dry") are cooled to below 5° C. and opened in an atmosphere of nitrogen. To each of bottles E and F there is 70 added 10 p.p.m. of dl- $\alpha$ -lipoic acid based on the ginger ale present. No modifier is added to bottle G. In bottles

E and G there are placed 5½" x ½" panels of black iron sheet prepared by sanding, followed by degreasing in refluxing trichloroethylene vapor. Into bottle F there is placed a similar black iron strip which is degreased in trichloroethylene vapor without prior sanding. The bottles are sealed without access of air and stored at room temperature. After one month no change is observable in the metal or liquid in samples E and F; whereas in sample G both the metal and the liquid are discolored.

*Example 4*

Two bottles of commercial ginger ale are cooled and opened in the absence of air as in Example 3. To bottle H there is added 35 p.p.m. of dl- $\alpha$ -lipoic acid. Bottle I is unmodified. Into each bottle is placed a 5½" x ½" black iron panel cleaned by degreasing in trichloroethylene vapor. The bottles are sealed and stored as in Example 3. After four days the metal in sample I is discolored. After four weeks the metal and liquid in sample H remain unchanged and the metal in sample I is black.

*Example 5*

Six 3" x 1" black iron panels are cleaned as in Example 2 and submerged respectively in the following liquids in loosely-capped glass containers:

| Sample | Liquid                                                       |
|--------|--------------------------------------------------------------|
| J      | 1% aqueous hydrochloric acid.                                |
| K      | 1% aqueous sulfuric acid.                                    |
| L      | water.                                                       |
| M      | 1% aqueous hydrochloric acid+0.1% dl- $\alpha$ -lipoic acid. |
| N      | 1% aqueous sulfuric acid+0.1% dl- $\alpha$ -lipoic acid.     |
| O      | water+0.1% dl- $\alpha$ -lipoic acid.                        |

A small fraction of the lipoic acid remains undissolved in samples M and N and is removed by filtration before inserting the panels. After 15 days at room temperature the condition of the panels and the liquids in the respective samples is as follows:

| Sample | Metal Panel          | Liquid                         |
|--------|----------------------|--------------------------------|
| J      | Loose, brown coating | clear.                         |
| K      | do                   | Do.                            |
| L      | Corroded             | cloudy, sediment in bottom.    |
| M      | Bright               | slightly cloudy, trace of ppt. |
| N      | do                   | Do.                            |
| O      | Trace of corrosion   | clear.                         |

After a total of five weeks and five months, respectively, at room temperature the panels in the respective samples are as follows:

| Sample | Metal Panels |                 |
|--------|--------------|-----------------|
|        | 5 Weeks      | 5 Months        |
| J      | Rusted       | Badly corroded. |
| K      | do           | Do.             |
| L      | Corroded     | Do.             |
| M      | Bright       | Bright.         |
| N      | do           | Do.             |
| O      | Rusted       | Badly corroded. |

Sample O shows that at pH about 7 this invention provides less corrosion resistance than at lower pH.

*Example 6*

Four 3" x 1" black iron panels are cleaned as in Example 2 and submerged respectively in the following liquids in loosely capped glass containers.

| Sample | Liquid                                                       |
|--------|--------------------------------------------------------------|
| P      | 5% aqueous hydrochloric acid.                                |
| Q      | 5% aqueous sulfuric acid.                                    |
| R      | 5% aqueous hydrochloric acid+0.1% dl- $\alpha$ -lipoic acid. |
| S      | 5% aqueous sulfuric acid+0.1% dl- $\alpha$ -lipoic acid.     |

Most of the lipoic acid dissolves in samples R and S. The slight excess is removed by filtration. The panels in the respective samples after three weeks and 4½ months at room temperature are as follows:

| Sample | Metal Panel              |                 |
|--------|--------------------------|-----------------|
|        | 3 Weeks                  | 4½ Months       |
| P      | Black coating            | Badly corroded. |
| Q      | Black (partly dissolved) | Do.             |
| R      | Bright                   | Bright.         |
| S      | do                       | Do.             |

The liquids in samples R and S remain clear and colorless after 4½ months of storage.

*Example 7*

Six black iron panels are cleaned as in Example 2 and inserted respectively in the following liquids in loosely-capped glass containers in such fashion that about ¼ of each panel is submerged and about ¼ remains in contact with the air above the liquid.

| Sample | Liquid                                                                           |    |
|--------|----------------------------------------------------------------------------------|----|
|        | 25                                                                               | 30 |
| T      | 10% aqueous hydrochloric acid.                                                   |    |
| U      | 10% aqueous hydrochloric acid+0.1% 5-(2-methyl-1,3-dithiane-4-yl)pentanoic acid. |    |
| V      | 10% aqueous hydrochloric acid+0.1% dl- $\alpha$ -lipoic acid.                    |    |
| W      | 10% aqueous sulfuric acid.                                                       |    |
| X      | 10% aqueous sulfuric acid+0.1% 5-(2-methyl-1,3-dithiane-4-yl)pentanoic acid.     |    |
| Y      | 10% aqueous sulfuric acid+0.1% dl- $\alpha$ -lipoic acid.                        |    |

All panels show corrosion in air above the liquids after one day. After one week and six weeks of storage at room temperature the submerged portions of panels in respective samples are as follows:

| Sample | Metal Panels     |                                              |
|--------|------------------|----------------------------------------------|
|        | One Week         | Six Weeks                                    |
| T      | Partly dissolved | Completely dissolved (liquid clear, yellow). |
| U      | Unchanged        | Unchanged (liquid slightly yellow).          |
| V      | do               | Unchanged (liquid colorless).                |
| W      | Black coating    | Completely dissolved (liquid clear, yellow). |
| X      | A few dark spots | A few corroded spots (liquid colorless).     |
| Y      | Unchanged        | Unchanged (liquid colorless).                |

When the following compounds are substituted for the  $\alpha$ -lipoic acid in Example 2, corrosion of black iron in contact with a commercial ginger ale is prevented:

- 5-(5-methyl-1,2-dithiolane-3-yl)pentanoic acid
- 6,8-dimercaptononanoic acid
- 5-(2-butyl-6-methyl-1,3-dithiane-4-yl)pentanoic acid
- 5-(1,5-dithiaspiro[5.5]hendecane-2-yl)pentanoic acid
- 5-(1,3-dithiane-4-yl)pentanamide
- 5-(2,2-diphenyl-1,3-dithiane-4-yl)pentanoic acid
- Sodium salt of 5-(1,3-dithiane-4-yl)pentanoic acid
- 5-(2,2-dimethyl-1,3-dithiane-4-yl)pentanoic acid
- Ethyl 5-(2-methyl-1,3-dithiane-4-yl)pentanoate
- 4-tert. butyl-5-(2-dithiolane-3-yl)pentanoamide
- 4-tert. butyl-6,8-dimercaptooctanoamide
- 2-(1,2-dithiolane-3-yl)acetic acid
- 3,5-dimercaptopenanoic acid
- 6-(1,2-dithiolane-3-yl)hexanoic acid
- 7,9-dimercaptonanoic acid
- 9-(1,2-dithiolane-3-yl)nonanoic acid
- 10,12-dimercaptododecanoic acid
- 4-ethyl-4-methyl-4-(1,2-dithiolane-3-yl)butyric acid
- 4-ethyl-4-methyl-5,7-dimercaptoheptanoic acid
- 9-(5-butyl-1,2-dithiolane-3-yl)nonanoic acid
- 10,12-dimercaptohexadecanoic acid

The above compounds may be used in this invention interchangeably with their lower alkyl esters, that is,

methyl, propyl, butyl esters and the like; amides; salts, particularly their sodium, potassium and ammonium salts; and similar carboxylic derivatives which are readily hydrolyzed to the corresponding acids. Of this group, the free acids and the salts are preferred because of their greater solubility in aqueous systems.

Of the organic compounds useful for reducing corrosion according to the present invention, a preferred group is composed of  $\alpha$ -lipoic acid, its reduction product, 6,8-dimercaptooctanoic acid, also known as gamma-lipoic acid, and the esters and salts of these acids. This group includes both the racemic forms of these compounds as well as their respective optical isomers when employed separately.

This preferred group of substituted 1,2-dithiolanes as well as the other organic compounds represented by the above formula R—R'—COR'', and their intermediates, can be prepared by one or more of the methods of assignee's U.S. Patents 2,752,249, 2,752,373, 2,752,374, 2,792,406, and 2,801,261.

The embodiments of the invention in which an exclusive property or privilege is claimed are defined as follows:

1. A method for reducing the corrosive effect of an acidic composition in contact with an iron-containing metal which comprises adding to said composition from 0.0001 to 10%, by weight of said composition, of an organic compound of molecular weight not exceeding 500 and of the formula



where R is a monovalent organic radical of the class consisting of



and the C-alkyl derivatives of these radicals wherein the alkyl groups are up to four carbons, R' is a divalent hydrocarbon radical of up to 8 carbon atoms, R''' and R'''

are members of the group consisting of hydrogen and hydrocarbon radicals of 1-10 carbon atoms and taken together represents a divalent hydrocarbon radical, and COR'' is selected from the class consisting of carboxyl and groups hydrolyzable thereto.

5 2. The method of claim 1 wherein the organic compound is  $\alpha$ -lipoic acid.

3. The method of claim 1 wherein the organic compound is 6,8-dimercaptooctanoic acid.

10 4. An iron-containing metal container having therein an acidic commodity and, as an inhibitor of corrosion from 0.0001 to 10% by weight of the commodity of an organic compound of molecular weight not exceeding 500 and of the formula



where R is a monovalent organic radical of the class consisting of



25 and the C-alkyl derivatives of these radicals wherein the alkyl groups are up to four carbons, R' is a divalent hydrocarbon radical of up to 8 carbon atoms, R''' and R''' are members of the group consisting of hydrogen and hydrocarbon radicals of 1-10 carbon atoms and taken together represent a divalent hydrocarbon radical, and COR'' is selected from the class consisting of carboxyl and groups hydrolyzable thereto.

30 5. The container of claim 4 in which the corrosion inhibitor is  $\alpha$ -lipoic acid.

35 6. The container of claim 4 in which the corrosion inhibitor is 6,8-dimercaptooctanoic acid.

#### References Cited in the file of this patent

#### UNITED STATES PATENTS

- 40 2,706,158 Searle \_\_\_\_\_ Apr. 12, 1955  
 2,752,249 Latham et al. \_\_\_\_\_ June 26, 1956